

## UNITED STATES PATENT OFFICE

2,196,992

## LIQUID POLISHING COMPOSITION

Edwin W. Keller, Allentown, Pa.

No Drawing. Application October 29, 1936,  
Serial No. 108,212

3 Claims. (Cl. 134—24)

This invention relates to polishes and particularly to an improved polish for use on bright metals including metal plating.

In the polishing of metals there are essentially two types of materials which must be removed from the metal to be polished. These are, first, the metallic compounds including metallic oxides and sulfides which are formed when the metal is exposed to the atmosphere, and, secondly, an accumulated surface film composed of dust, oil and the like. Heretofore, many polishes for use on bright metals have been unsatisfactory because they failed to remove the external surface film of dust or oil. Other polishes which accomplish the removal of the surface film by means of various alkali substances are objectionable because they leave a film which is caused by the action of fatty acid soaps or the like or solvents present in the polish. Moreover, where fatty acid soaps are used there is the further difficulty of a tendency for the polish to turn rancid. Another disadvantage inherent in many of the prior art liquid polishes is the tendency to form a hard cake on standing, thus necessitating vigorous and prolonged shaking before the polish can be used. Moreover, most polishes are unsatisfactory because of the inclusion of ingredients which are so abrasive as to scratch a smooth metal surface. Furthermore, some of the prior art polishes have toxic properties as well as disagreeable odors.

One of the most serious difficulties encountered in the preparation of metal polishes has to do with the formation of a hard cake of material when the polish is allowed to stand. The term "hard cake" as used throughout this specification refers to a conglomerate which can be re-distributed by shaking only with much difficulty if at all and is to be distinguished from soft settling which can be re-distributed easily by shaking.

The principal object of the present invention is to provide a liquid polish which will be substantially free from the formation of a hard cake. A further object is to provide a polish which will remove surface film without leaving a film caused by ingredients in the polish. A still further object is to provide a polish which is free from ingredients of high abrasive power.

In the development of the present invention I have proceeded in accordance with the following theory which I have evolved after an extended investigation of the problem. An abrasive alone is not sufficient in view of the two different types of materials that a polish must remove and in view of the fact that most abrasives settle.

Therefore an assistant ingredient with detergent properties as well as suspending properties must be used and this ingredient must not include highly alkaline substances else an alkali film will form after the polish is used. Sodium silicate, well known as a detergent, also has the property of assisting in the suspension of finely divided abrasives. Finally a third ingredient is necessary for the prevention of the formation of a hard cake due to the natural affinity of the abrasive and its assistant. This third ingredient must coat with the abrasive substance so as to substantially prevent a hard-caking effect caused by the affinity of the assistant for the abrasive and at the same time it must be compatible with both the abrasive and its assistant.

I have discovered that finely divided tin oxide in a substantially pure state is an admirable abrasive for bright metals including metal plating since its polishing qualities are good while its abrasive qualities are such as to preclude scratching. However, a suspension of tin oxide in water is not a satisfactory polish where the surface to be cleaned has acquired a film of dirt, oil or the like. Where such conditions prevail, tin oxide alone is not capable of cutting through the surface film. Moreover, a suspension of tin oxide alone is not suitable as a polish due to the fact that the particles of tin oxide settle rapidly to the bottom of the container. However, the difficulties connected with the use of a suspension of tin oxide alone can be partially overcome by the use of sodium silicate which acts as a detergent for the surface film of dirt, oil or the like and at the same time contributes to maintaining a suspension of the particles of tin oxide. As already generally stated with respect to finely divided abrasives and assistant detergents like sodium silicate, a marked tendency for the sodium silicate to combine physically with the particles of tin oxide in such a way as to form a hard cake of material within the container, necessitating an undue amount of shaking before the polish can be used. According to the present invention, this difficulty of the formation of a hard cake is substantially obviated by the use of a third ingredient which not only acts substantially to prevent the formation of a hard cake, but also aids the sodium silicate in the attack on the surface film and at the same time has the remarkable quality of retarding the tarnishing of the metallic surface which is polished. This added ingredient is marketed under a number of trade names such as "Gardinol," "Duponol" and "Orvus," but these products are substantially the

same, their principal active ingredient being the sodium salt of lauryl alcohol sulfate. The prevention of the formation of a hard cake by this added ingredient, hereinafter referred to as 5 "Duponol," is apparently effected by the action of lauryl alcohol sulfate upon the particles of tin oxide which appear to be insulated by the "Duponol" from the cohesive action of the sodium silicate. It is also important to note that "Duponol" 10 and sodium silicate are compatible as well as completely rinsable from the polished surface. Moreover, "Duponol" is a neutral compound and does not hydrolyze to give an alkaline reaction.

One of the preferred ways of carrying out the 15 present invention is as follows: Three grains of powdered "Duponol," preferably "Duponol M. E. Dry," are added to four gallons of water and agitated until completely dissolved. To eight ounces of the "Duponol" solution so obtained 20 eight pennyweight of tin oxide is added and the mixture thoroughly agitated. To the mixture so obtained three c. c. of sodium silicate is then added and after a thorough agitation the resultant polish is ready for use. I have discovered 25 that the maximum inhibition of caking is obtained when the mixture of "Duponol" and tin oxide abrasive is made prior to the addition of the sodium silicate detergent. The results obtained by mixing in this order are far superior 30 to the results obtained when the sodium silicate is mixed with the "Duponol" solution prior to the addition of the tin oxide.

The sodium silicate mentioned above is preferably one having an alkali to silica ratio of 35 about 1:3.86 corresponding to a density of 33.5° Baumé, but of course it will be understood that silicates of different ratios may be used to advantage provided the alkali ratio is kept relatively low. It is to be understood, however, that the 40 silicates used in the practice of this invention

are not to be confused with certain abrasive silicon dioxide compounds, such as silex, which have heretofore been used in some polishes.

The polish prepared as above described may be applied by rubbing a small quantity of it on the 5 material to be polished, allowing the polish to dry slightly, and removing the residue with a soft cloth. Remarkable results are obtained with a minimum of effort and retarnishing is noticeably inhibited. 10

While the present invention has been described in detail with reference to a specific polishing composition, it is to be understood that various changes in the amounts of the ingredients used are within the contemplation of the invention 15 and should not be deemed to constitute a departure from the spirit of the invention as hereinafter claimed.

Having thus described my invention, I claim:

1. An aqueous liquid polishing composition 20 comprising finely divided tin oxide, sodium silicate, as a detergent, having a low alkali silica ratio, so that an objectionable alkali film will not form on the polished work, and the sodium salt of lauryl alcohol sulfate for preventing hard 25 caking of the aforesaid ingredients on standing, besides assisting the detergent action of the sodium silicate and retarding tarnishing of metal surfaces polished with the composition.

2. A liquid polishing composition as set forth 30 in claim 1 further characterized in that the sodium silicate has an alkali silica ratio substantially corresponding to a density of 33.5° Baumé.

3. A method of preparing the composition set 35 forth in claim 1 which comprises first mixing the tin oxide and the lauryl alcohol sulfate together in water, and thereafter adding and mixing in the sodium silicate.

EDWIN W. KELLER. 40